

## UNITED STATES PATENT OFFICE

2,381,406

## ALIPHATIC DINITRO TETRANITRATES

Henry B. Hass, West La Fayette, Ind., and Wilbur R. McElroy, Beacon, N. Y., assignors to Purdue Research Foundation, La Fayette, Ind., a corporation of Indiana

No Drawing. Application July 29, 1944,  
Serial No. 547,285

## 4 Claims. (Cl. 260—467)

Our invention relates to new compositions of matter. More particularly it is concerned with aliphatic dinitro tetranitrates having the following structural formula:



in which  $n$  represents an integer less than 5.

As examples of compounds contemplated by the present invention, there may be mentioned 2,4-bis-(hydroxymethyl)-2,4-dinitro-1,5-pentanediol

copending application, U. S. Serial No. 547,284, filed July 29, 1944. By the procedure there described, the desired dinitroalkane is reacted with formaldehyde in a ratio of four moles of the latter to one of dinitroalkane. The reaction is effected in the presence of an alkaline catalyst such as calcium hydroxide and a suitable solvent such as ethanol. The temperature of the reaction mixture should preferably be held at about 20° C.

In the table appearing below some of the various physical properties of certain aliphatic dinitro tetranitrates covered by the present invention are listed.

Table

| Compound                                                            | Melting point, °C | Percent nitrogen |       | Percent nitrogen (ester) |       | Percent carbon |       | Percent hydrogen |       |
|---------------------------------------------------------------------|-------------------|------------------|-------|--------------------------|-------|----------------|-------|------------------|-------|
|                                                                     |                   | Calc'd.          | Found | Calc'd.                  | Found | Calc'd.        | Found | Calc'd.          | Found |
|                                                                     |                   |                  |       |                          |       |                |       |                  |       |
| 2, 5-bis (hydroxymethyl)-2, 5-dinitro-1, 6-hexanediol tetranitrate  | 132-134           | 18.75            | 16.80 | 12.5                     | 12.2  | 21.44          | 23.5  | 2.69             | 3.8   |
| 2, 6-bis (hydroxymethyl)-2, 6-dinitro-1, 7-heptanediol tetranitrate | 84-85             | 18.18            | 16.86 | 12.1                     | 11.9  | 23.38          | 24.4  | 3.05             | 3.    |
| 2, 7-bis (hydroxymethyl)-2, 7-dinitro-1, 8-octanediol tetranitrate  | 128-129           |                  |       |                          |       |                |       |                  |       |

tetranitrate, 2,5-bis(hydroxymethyl) 2,5-dinitro-1,6-hexanediol tetranitrate, 2,6-bis(hydroxymethyl) 2,6-dinitro-1,7-heptanediol tetranitrate, 2,7-bis(hydroxymethyl) 2,7-dinitro-1,8-octanediol tetranitrate, and the like.

Compounds of the above type are readily prepared by subjecting the corresponding aliphatic dinitro tetrol to nitration in the liquid phase, utilizing as the nitrating agent a mixture of sulphuric and nitric acids. Generally the acid mixture employed usually consists of about five parts of sulphuric acid and three parts of nitric acid by weight. A quantity of the mixed acids, eight times the weight of tetrol to be nitrated, is placed in a suitable reaction vessel which is immersed in ice. The tetrol is slowly added in portions to the acid mixture while agitating. After the entire amount of tetrol has been added in this manner, agitation is continued for a short time and thereafter the contents of the reaction vessel are poured into a large volume of ice water. The tetranitrate then separates as an insoluble product. Further purification of the material thus obtained may be effected by recrystallization from methanol or other suitable solvents.

The tetrols employed in preparing the compounds of the present invention are prepared in accordance with the procedure described in our

identification of these compounds, it is to be understood that we do not desire to limit ourselves to products having the exact physical properties listed since the data were obtained from single preparations of the various compounds given above.

The aliphatic dinitro tetranitrates of our invention are useful as explosives. Additional uses of these compounds will be apparent to those skilled in the art.

Our invention now having been described, what we claim is:

1. Aliphatic dinitro tetranitrates of the formula:



in which  $n$  represents an integer less than 5.

2. 2,5-bis(hydroxymethyl) 2,5-dinitro-1,6-hexanediol tetranitrate.

3. 2,6-bis (hydroxymethyl) 2,6-dinitro-1,7-heptanediol tetranitrate.

4. 2,7-bis (hydroxymethyl) 2,7-dinitro-1,8-octanediol tetranitrate.

HENRY B. HASS.  
WILBUR R. McELROY.

CERTIFICATE OF CORRECTION.

Patent No. 2,381,406.

August 7, 1945.

HENRY B. HASS, ET AL.

It is hereby certified that error appears in the printed specification of the above numbered patent requiring correction as follows: Page 1, in the table, under the heading "Percent hydrogen", for "3." read --3.8--; and that the said Letters Patent should be read with this correction therein that the same may conform to the record of the case in the Patent Office.

Signed and sealed this 25th day of December, A. D. 1945.

Leslie Frazer

(Seal)

First Assistant Commissioner of Patents.